

## UNITED STATES PATENT OFFICE

2,688,595

## LUBRICANTS

Morton Fainman, Chicago, Ill., assignor to Standard Oil Company, Chicago, Ill., a corporation of Indiana

No Drawing. Application November 23, 1949,  
Serial No. 129,170

7 Claims. (Cl. 252—34)

1

This invention is directed to improvements in oleaginous compositions and more particularly relates to stable, corrosion and/or rust inhibiting hydrocarbon oil compositions.

Organic substances such as normally nongaseous hydrocarbon products, particularly petroleum products, such as lubricating oils, turbine oils, insulating oils, greases, waxes and non-viscous petroleum products, such as naphthas, gasolines, fuel oils, as well as synthetic hydrocarbon oils, are susceptible to oxidative deterioration. This oxidation takes place under prolonged storage at atmospheric temperatures, as well as during use under elevated temperatures. Oxidative deterioration of this type is also encountered with fats and fatty materials, such as animal, vegetable and marine oils, for example, cottonseed oil, corn oil, lard oil, tallow, menhaden oil, etc.

In many types of machinery and industrial equipment in which water or steam or other aqueous liquids are used which may become contaminated with such aqueous media, rusting and/or corrosion of the metal parts is encountered although oil may come in contact with such metal parts. For example, in internal combustion engines, water due to condensation accumulates and causes rusting and/or corrosion of the ferrous metal parts of such engines. In the operation of steam turbines, rusting or corrosion of the ferrous metal parts of such systems is also a serious problem and the prevention or inhibition of such rusting and/or corrosion is highly important. Corrosion is also a serious problem in the operation of textile machinery, in shock absorbers, in hydraulic lifts, etc. Although equipment of the foregoing type usually employ an oil of some sort, the oil film which may form on the metal surfaces does not provide adequate protection against rusting and/or corrosion by the aqueous media due to the partial displacement of this oil film from the metal surfaces.

It is an object of the present invention to provide organic compositions which are resistant to oxidative deterioration and which prevent corrosion and/or rusting of metal surfaces. Another object of the invention is to provide a composition containing an oleaginous material which is resistant to oxidative deterioration and which will prevent the rusting and/or corrosion of metal surfaces with which it comes in contact. A further object of the present invention is to provide compositions containing petroleum products which are resistant to oxidative deterioration and which are also effective in preventing rusting and/or

2

corrosion of metal surfaces coated with a film of said petroleum composition. Still another object of the invention is to provide a petroleum oil composition which is resistant to deterioration due to oxidation and which is capable of preventing rusting and/or corrosion of metal surfaces in contact with such petroleum oil compositions. Other objects and advantages will become apparent from the following description thereof.

I have discovered that the foregoing objects can be attained by incorporating in organic compositions of the type hereinafter described, particularly petroleum products, such as petroleum oils, a small amount, sufficient to inhibit oxidative deterioration and to inhibit rusting and/or corrosion, of an oil-soluble ammonium salt of an arylol acid ether obtained by reacting equimolar proportions of an amine and an arylol acid ether at a temperature of from about 50° F. to about 300° F., and preferably from about 150° F. to about 250° F. The amine used is preferably an amino compound known to possess antioxidant properties, particularly the aromatic amino compounds, such as for example, p-amino phenyl-beta-naphthylamine, N-phenyl-p-phenylene diamine, p-amino acetinalide, o-phenylene diamine, m-phenylene diamine, p-phenylene diamine, benzidine, p,p'-diamino diphenyl methane, etc., and alkylene diamines, such as for example, 1,2-diamino ethane, 1,2-diamino butyl ethane, propylene polyamine, ethylene diamine, etc.

The arylol acid ether is preferably one having the general formula



wherein R and R' are substituents selected from the group consisting of hydrogen or an alkyl group, A is a substituent selected from the group consisting of hydrogen or the group



wherein R and R' are as above, R'' is a substituent selected from the group consisting of hydrogen, aryl, alkyl, aralkyl, alkaryl, and mixtures thereof, and n is an integer of from 1 to 4, inclusive, and wherein R plus R' contains 10 to 30 carbon atoms. R, R' and R'' may be the same or different alkyl radicals. In the above formula

the ring structure represents a mono- or poly-nuclear aryl nucleus, such as phenyl, naphthyl, etc. groups.

The preferred compounds are those in which "A" is hydrogen and  $n$  is 1 or 2.

Representative of specific examples of compounds coming within the above general formula are the following:

Catechol mono-alpha-stearic acid ether  
 Catechol di-alpha-stearic acid ether  
 Resorcinol mono-alpha-stearic acid ether  
 Hydroquinone mono-alpha-stearic acid ether  
 Hydroquinone di-alpha-stearic acid ether  
 Naphthalene-1,5-di-alpha-stearic acid ether  
 Phloroglucinol mono-alpha-stearic acid ether  
 Phloroglucinol di-alpha-stearic acid ether  
 Phloroglucinol tri-alpha-stearic acid ether  
 Catechol mono-alpha-lauric acid ether  
 Resorcinol lauric stearic acid ether  
 Hydroquinone di-palmitic acid ether  
 Catechol mono-alpha-oleic acid ether  
 Resorcinol mono-montanic acid ether  
 Phloroglucinol mono-behenic acid ether  
 Catechol mono-linoleic acid ether  
 Pyrogallol mono-stearic acid ether

The ammonium salts of arylol acid ethers are exemplified by the following compounds:

Di-butyl-p-phenylene diamine-2-hydroxyphenoxy-alpha-stearate  
 Para-amino phenyl- $\beta$ -naphthylammonium-alpha-alpha-dihydroxy-phenoxy stearate  
 Phenyl-alpha-naphthylammonium-alpha - para-dihydroxyphenoxy stearate  
 1-2-diamino ethane - ortho - dihydroxyphenoxy oleate  
 Ethylene diamine sym-trihydroxyphenoxy behenate  
 Para-amino-acetanilide - alpha - ortho - dihydroxy-phenoxylaurate  
 Butylethanolammonium-2-hydroxy-phenoxy-alpha-stearate, etc.

100° F. of about 100 seconds to 350 seconds are employed. With the advent of drastic refining treatments to produce more highly refined turbine oils having improved color, etc., desirable components for preventing the oxidative deterioration of the oils and these responsible for the wetting and therefore rust inhibiting qualities of the oil are removed. To overcome the susceptibility of such oils to oxidative deterioration and 10 to impart rust inhibiting properties thereto, small amounts, of the order above stated, of the reaction product of an amine and an arylol acid ether is added to the turbine oil. To determine the effectiveness of such additives in providing a turbine oil which is resistant to oxidation and which is effective in inhibiting rusting or corrosion, a turbine oil comprising a highly refined mineral oil having a Saybolt Universal viscosity at 100° F. of about 160 seconds was compounded with 0.1% 15 of various ammonium salts of the present invention and subjected to the following oxidation test: The oil composition is heated and maintained at a temperature of about 150° F. while blowing oxygen therethrough, and at stated periods a sample of the oil is withdrawn to determine the neutralization number thereof, and the test continued for 336 hours or until a sample has a neutralization number of 2. The neutralization number is determined by adding two 20 grams of the sample to a neutral solution of 200 cubic centimeters of naphtha and 100 cubic centimeters of 95% ethyl alcohol containing phenolphthalein. The mixture is then titrated with N/10 sodium hydroxide to the first pink color. 25 The neutralization number is calculated from the equation:

$$\text{Neutralization No.} = \frac{\text{c. c. NaOH} \times \text{normality} \times 56.1}{\text{Weight of sample}}$$

The data obtained in the foregoing test are tabulated in Table I.

TABLE I  
*Oxidation test*

| Sample No.                                                                               | Time Until Neutralization No. of Sample Equals 2 | Appearance of Sample After Test |
|------------------------------------------------------------------------------------------|--------------------------------------------------|---------------------------------|
| 1—Control (no additive)                                                                  | Hours                                            |                                 |
| 2—Control+1% 2-hydroxy phenoxy-alpha-stearic acid.                                       | 8                                                | Red-brown sludge.               |
| 3—Control+1% di-butyl-p-phenylene di-amine-2-hydroxy-phenoxy-alpha-stearate.             | 20                                               | No sludge.                      |
| 4—Control+1% P-amino phenyl- $\beta$ -naphthylammonium-2-hydroxy phenoxy-alpha-stearate. | 160                                              | Do.                             |
| 5—Control+1% Phenyl-alpha-naph-thyl ammonium - 2 - hydroxy phenoxy-alpha-stearate.       | 336                                              | Do.                             |
|                                                                                          | 320                                              | Do.                             |

It is not intended to imply that all amine salts of arylol acid ethers serve with identical efficiency; while they are all effective, they will exhibit some variation depending upon the nature and severity of the service to which they are subjected. In general, it will be found that from about 0.0005% to about 2.0%, and preferably from about 0.003% to about 0.5% by weight of the ammonium salt of arylol acid ether will provide adequate protection.

For the purpose of illustrating the present invention the same will be described as applied to steam turbine lubrication for which highly refined oils having Saybolt Universal viscosities at

65 100° F. of about 100 seconds to 350 seconds are employed. With the advent of drastic refining treatments to produce more highly refined turbine oils having improved color, etc., desirable components for preventing the oxidative deterioration of the oils and these responsible for the wetting and therefore rust inhibiting qualities of the oil are removed. To overcome the susceptibility of such oils to oxidative deterioration and 10 to impart rust inhibiting properties thereto, small amounts, of the order above stated, of the reaction product of an amine and an arylol acid ether is added to the turbine oil. To determine the effectiveness of such additives in providing a turbine oil which is resistant to oxidation and which is effective in inhibiting rusting or corrosion, a turbine oil comprising a highly refined mineral oil having a Saybolt Universal viscosity at 100° F. of about 160 seconds was compounded with 0.1% 15 of various ammonium salts of the present invention and subjected to the following oxidation test: The oil composition is heated and maintained at a temperature of about 150° F. while blowing oxygen therethrough, and at stated periods a sample of the oil is withdrawn to determine the neutralization number thereof, and the test continued for 336 hours or until a sample has a neutralization number of 2. The neutralization number is determined by adding two 20 grams of the sample to a neutral solution of 200 cubic centimeters of naphtha and 100 cubic centimeters of 95% ethyl alcohol containing phenolphthalein. The mixture is then titrated with N/10 sodium hydroxide to the first pink color. 25 The neutralization number is calculated from the equation:

$$\text{Neutralization No.} = \frac{\text{c. c. NaOH} \times \text{normality} \times 56.1}{\text{Weight of sample}}$$

The data obtained in the foregoing test are tabulated in Table I.

time the steel specimen is removed from the beaker, washed with naphtha and visually inspected for the presence of rust. Samples of a turbine oil base, namely a hydrocarbon oil having a Saybolt Universal viscosity at 100° F. of about 150 seconds containing small amounts of various salts of the type herein described were subjected to this test and the results obtained tabulated in Table II.

TABLE II

| Additive                                                                      | Percent Present | Degree of Rust        |
|-------------------------------------------------------------------------------|-----------------|-----------------------|
| 1—None                                                                        |                 |                       |
| 2—P-amino phenyl- $\beta$ -naphthylammonium-2-hydroxy phenoxy-alpha-stearate. | 0.003           | Extreme, Very slight. |
| 3—Phenyl- $\alpha$ -naphthylammonium-2-hydroxy phenoxy-alpha-stearate.        | 0.003           | Slight.               |
| 4—Di-butyl-p-phenylene diamine-2-hydroxy phenoxy-alpha-stearate.              | 0.001           | Very slight.          |
| 5—Di-butyl-p-phenylene diamine-2-hydroxy phenoxy-alpha-stearate.              | 0.003           | None.                 |
| 6—Di-butyl-p-phenylene diamine-2-hydroxy phenoxy-alpha-stearate.              | 0.005           | Do.                   |
| 7—Di-butyl-p-phenylene diamine-2-hydroxy phenoxy-alpha-stearate.              | 0.01            | Do.                   |

The above data demonstrate the effectiveness of very small amounts of the additives in the present invention in inhibiting rusting.

Compositions containing the herein described ammonium salts of arylol acid ether can also contain in addition pourpoint depressors, extreme pressure agents, viscosity improvers, detergents, etc.

While I have described my invention by reference to a specific embodiment thereof, the invention is not limited thereto, but includes within its scope such modifications and variations as come within the spirit of the appended claims.

I claim:

1. A composition comprising essentially a major proportion of an oil and an oil-soluble aromatic amino salt obtained by reacting an arylol carboxylic acid ether with an aromatic amino compound selected from the class consisting of a naphthylamine, a phenylenediamine and pp' diamino diphenyl methane, said salt being used in small but sufficient amounts to inhibit the oxidative deterioration of said oil and to impart a corrosion-inhibiting property to said oil.

2. A composition as described in claim 1 in which the arylol carboxylic acid ether has the general formula



wherein R and R' are substituents selected from the group consisting of hydrogen and an alkyl group, A is a substituent selected from the group consisting of hydrogen and the group



in which R and R' are as above described, R'' is a substituent selected from the group consisting of hydrogen, aryl, alkyl, aralkyl, alkaryl radicals, and mixtures thereof, n is an integer of from 1 to 4, inclusive and wherein R plus R' contain from about 10 to about 30 carbon atoms.

3. A composition comprising essentially a normally non-gaseous petroleum fraction and from about 0.0005% to about 2.0% of an oil-soluble aromatic amino salt obtained by reacting an arylol carboxylic acid ether with an aromatic amino compound selected from the class consisting of a naphthylamine, a phenylenediamine and a pp' diamino diphenyl methane.

4. A composition as described in claim 3 in which the arylol carboxylic acid ether is an arylol stearic acid ether.

5. A composition comprising essentially a hydrocarbon oil and from about 0.0005% to about 2.0% of di-butyl-para-phenylenediamine-2-hydroxy-phenoxy-alpha-stearate.

6. A composition comprising essentially a hydrocarbon oil and from about 0.0005% to about 2.0% of para-amino phenyl-beta-naphthylammonium-2-hydroxy-phenoxy-alpha-stearate.

7. A composition comprising essentially a hydrocarbon oil and from about 0.0005% to about 2.0% of phenyl-alpha-naphthylammonium-2-hydroxy-phenoxy-alpha-stearate.

#### References Cited in the file of this patent

#### UNITED STATES PATENTS

| Number    | Name               | Date          |
|-----------|--------------------|---------------|
| 2,198,293 | Reiff et al. ----- | Apr. 23, 1940 |
| 2,252,665 | Reiff et al. ----- | Aug. 12, 1941 |
| 2,426,496 | Farley -----       | Aug. 26, 1947 |
| 2,447,483 | Baker -----        | Aug. 24, 1948 |
| 2,459,717 | Perry -----        | Jan. 18, 1949 |
| 2,470,276 | Watkins -----      | May 17, 1949  |

#### OTHER REFERENCES

"Lubricating Oil Additives," by Kalichevsky, in Petroleum Refiner, vol. 28, No. 10, pages 127 and 128.

Polar Type Rust Inhibitors, I. and E. Chem., vol. 40, No. 12, pages 2338 to 2347, page 2343 pertinent.